# EUROPEAN PATENT SPECIFICATION

(11) **EP 0 109 740 B1**
(45) Date of publication and mention of the grant of the patent: **09.03.1988**
(21) Application number: 83305660.9
(22) Date of filing: 23.09.1983
(51) Int. Cl.: C10L 1/32

(54) **Combustible compositions containing coal, water and surfactant**
Brennbare Zusammensetzungen die Kohle, Wasser und einen Surfaktant enthalten
Compositions combustibles contenant du charbon, de l'eau et un agent tensioactif

(30) Priority: 22.10.1982 GB 8230235
(43) Date of publication of application: 30.05.1984
(73) Proprietor: IMPERIAL CHEMICAL INDUSTRIES PLC, London SW1P 3JF (GB)
(72) Inventor: Bognolo, Guido, B-3078 Everberg (BE); Tadros, Tharwat Fouad, Wokingham Berkshire (GB)
(74) Representative: James, David Gomer

(56) References cited:
- EP-A- 0 057 576
- WO-A-83/04044
- GB-A- 1 179 572

## Description

This invention relates to stabilised aqueous slurries of pulverised coal, more particularly to such slurries which are stabilised by means of specified agents, which are valuable aids towards achieving the optimum fuel utilisation of coal.

With the increasing cost and anticipated eventual scarcity of crude oil and its refined products, renewed emphasis is being placed on the use of coal as a fuel. The physical form of coal, however, places severe limitations on its direct use if this is to be done in an efficient and environmentally acceptable manner, and consequently several techniques are currently being explored whereby these limitations may be overcome or minimised. Mention may be made, for example, of coal gasification processes and the reduction of the coal to finely divided form in suspension in oil, methanol or water. Coal-in-water slurries, in particular, offer a number of conceptual and practical advantages, notably low cost, ease of handling and low transportation costs as compared with dry pulverised coal, comparatively high burning efficiency and lower ash yield after combustion. The slurries are prepared by admixing the finely pulverised coal with water, usually in the presence of dispersing agents and suspension stabilisers. The role of the dispersing agent is to prevent floculation or coagulation of the coal particles during the mixing process, whilst the suspension stabiliser serves to prevent settling out of the dispersed particles on storage pf the slurry. Clearly, for economic reasons, it is desirable to maximise the coal content of the slurries, so as to minimise the absorption of heat due to evaporation of the water during combustion. High coal solids contents, however, generally lead to the slurries having extremely high viscosities, which in turn render very difficult or impossible the handling and transfer of the slurries, especially by pumping.

In EP-A-0057576 there is disclosed a dispersion of coal in water which contains, as a dispersant, a polyalkylene oxide nonionic surfactant which contains, in the hydrophilic portion thereof, at least 100 ethylene oxide units. One class of surfactant which can be used as a dispersant is a glycol ether of an alkyl phenol of a specified general formula. This dispersant contains only ethylene oxide units in the polyalkylene oxide chain. Another class of surfactant is a poly(oxyethylene)-poly(oxypropylene)-poly-(oxyethylene) block polymer. Yet a further class of surfactant is an alkylene diamine having polyalkylene oxide chains which are polyalkylene oxide and polyethylene oxide blocks and which are attached to the nitrogen atoms of the diamine. It is an essential feature of all of these various types of surfactant that they contain a total of at least 100 ethylene oxide units.

WO-A-83/04044, which is not a prior publication and falls within the terms of Art 54(3) EPC, discloses an aqueous slurry of a pulverised carbonaceous material and a water-soluble surface active alkylene oxide adduct of the formula: where R is an aliphatic, acyl or substituted aryl group and n has a value of at least 40. The essential feature of this prior application is the use of a surface active additive which is a polyethylene oxide derivative. The use of additives containing propylene oxide units does not form a part of the invention of this non-prior published application, although the use of certain materials of this type is exemplified by way of comparison.

We have now found that, through the use of certain defined dispersing agents which contain both propylene oxide and ethylene oxide units, coal-in-water slurries of high coal content can be prepared which nevertheless have viscosities low enough to avoid or minimise the problems of handling and transfer of slurries having a high coal solids content.

According to the present invention we provide a combustible composition consisting of a stabilised suspension of pulverised coal in water, the composition comprising
(i) from 30 to 90 parts by weight of pulverised coal,
(ii) from 0.05% to 3%, based on the dry weight of the pulverised coal, of a dispersing agent having the general formula: wherein R is an alkyl group containing from 5 to 22 carbon atoms, or an alkylphenyl group in which the alkyl group contains from 5 to 22 carbon atoms, x is an integer from 3 to 30 and y is an integer at least 10, and
(iii) sufficient water to. bring the total composition weight to 100 parts.

The dispersing agents used are thus block copolymer condensates of aliphatic alcohols or alkylphenols with propylene oxide and ethylene oxide respectively. The poly(oxyethylene) block occupies the terminal position in the poly(oxyalkylene) chain. The group R in formula (I) may be a linear or branched alkyl group containing from 5 to 22 carbon atoms, preferably 16 to 20 atoms, for example the mixed C,₆/C,ₑ alkyl groups derived from commercial stearyl alcohol. Alternatively, the group R may be a linear or branched chain alkylphenyl group in which the alkyl group contains from 5 to 22 carbon atoms preferably 6 to 12 carbon atoms, for example a hexyl, octyl, nonyl or dodecyl group.

Preferably the value of x in formula (I) is 10 to 20, and the value of y is 10 to 150, for example 80 to 120.

The dispersing agents are readily obtained by the successive reaction of the appropriate aliphatic alcohol or of nonylphenol successively with propylene oxide and with ethylene oxide.

The proportion of dispersing agent used preferably lies in the range 0.5% to 1.5% of the dry weight of the coal in the composition; there may be used either a single dispersing agent or a mixture of two or more agents as defined.

The pulverised coal for incorporation in the compositions of the invention may be obtained by techniques already well known such as by the use of tumbling mills or ball mills with recirculation of the ground material until the desired particle size distribution is obtained. The particle size of the coal is not critical for the purposes of the invention, but the preferred grade is that in which at least 80% of the particles are of a size below 75 micrometres.

.As already stated, the coal content of the compositions may vary between 30 parts and 90 parts by weight out of a total composition weight of 100 parts; more typically, it will lie in the range 50 parts to 80 parts by weight.

The dispersing agents as hereinabove defined are in general effective not only in facilitating the initial dispersing of the coal in the water but also in stabilising the dispersions against settling out of the coal particles on storage. However, if desired, the compositions of the invention may also contain conventional suspending or anti-settling agents.

The compositions are conveniently prepared by the steps of
(a) dissolving or dispersing the dispersing agent in the water,
(b) adding the pulverised coal and
(c) subjecting the mixture to the action of a mixer for a sufficient period of time to produce a dispersion, usually of the order of 2 minutes using a high speed mixer. It is normally satisfactory to carry out these operations at or near room temperature. In certain cases, it may be desirable to add an anti-foaming agent to prevent excessive foam formation during the mixing operation.

The compositions of the invention exhibit substantially lower viscosities at comparable coal solids contents than do known coal-in-water slurries prepared with the aid of conventional surfactants such as sodium or calcium lignin sulphonates or condensed naphtalene-formaldehyde sulphonates or sodium polyacrylates. They also show improved stability towards settling out of the coal particles on storage. They are therefore very suitable for use as fuels in process heaters and in industrial and other types of boiler.

The invention is illustrated by the following examples, in which parts and percentages are by weight.

### Examples

### General procedure

The dispersing agent indicated was dissolved or dispersed in water to yield the stated concentration based on dry weight of coal, and to the solution or dispersion was added pulverised coal in the stated proportion; the mixture was then subjected to the action of a high-speed mixer for 2 minutes. After each slurry had stood for approximately 15 minutes at room temperature to permit deaeration, its viscosity was measured on a Brookfield viscometer (immediately before measurement, each sample was homogenised by gentle hand stirring).

The coal samples used in certain of the Examples had the following characteristics:

For comparison, the procedure was repeated in the absence of the dispersing agent as herein defined and also, in certain instances, with the dispersing agent replaced by an equal amount of a conventional anionic surfactant. The compositions of the slurries and their viscosities are shown in the individual Examples.

### Example 1

### Coal sample: No. 1

Dispersing agent: Agent A (nonylphenol condensed successively with 15.5 molar proportions of propylene oxide and 33 molar proportions of ethylene oxide).

### Example 2

### Coal sample: No. 2

Dispersing agent: Agent A, as in Example 1.

### Example 3

### Coal sample: No. 1

Dispersing agent: Agent B (nonyl phenol condensed successively with 16 molar proportions of propylene oxide and 120 molar proportions of ethylene oxide).

### Example 4

### Coal sample: No. 3

Dispersing agents: Agent A and B as in Examples 1 and 3.

### Example 5

Coal sample: a non-beneficiated coal having an ash content of 15-20% by weight and an inorganic sulphur content of 2-4% by weight. 80% of the particles were of a size below 75 micrometres.

Dispersing agents: Agent C (nonylphenol condensed successively with 7.4 molar proportions of propylene oxide and 28.0 moles of ethylene oxide).

Agent D (nonylphenol condensed successively with 7.6 molar proportions of propylene oxide and 45.5 moles of ethylene oxide).

### Example 6

### Coal sample: a beneficiated coal; 80% of the particles were of a size below 75 micrometres.

Dispersing agent: Agent D, as in Example 5.

### Example 7 .

### Coal sample: a non-beneficiated coal; 75.8% of the particles were of a size below 75 micrometres.

Dispersing agents: Agent E (commercial stearyl alcohol condensed successively with the 15 molar proportions of propylene oxide and 100 molar proportions of ethylene oxide).

Agent A, as in Example 1:

### Example 8

### Coal sample: Coal sample No. 3 as described above was used for this series of experiments.

Dispersing agents: Agent F (nonylphenol condensed successively with 13.5 molar proportions of propylene oxide and 30 molar proportions of ethylene oxide.) Agent G (oleyl alcohol condensed successively with 15 molar proportions of propylene oxide and 100 molar proportions of ethylene oxide.)

For comparative purposes, to show the advantage of using block copolymer additives, tests were carried out using polymers containing only ethylene oxide.

### Agent H (nonylphenol condensed with 30 molar proportions of ethylene oxide.) Agent I (stearyl alcohol condesned with 100 molar proportions of ethylene oxide.)

Dispersions were made up using 1 % (based on dry weight of coal) and viscosity was measured with a Brookfield viscometer at 0.5 rpm using a No. 3 spindle.

Comparison of the results with Agents F and H shows that a reduced viscosity at 65% coal content is obtained using the block copolymer compared with the simple ethoxylate at the same coal content. At 68% coal content the composition containing the simple ethoxylate is unusable.

Comparison of the results obtained using Agents G and I shows that use of the block copolymer allows a higher solids content than with the simple ethoxylate. Thus additives of general formula (I) in which R is a C₁₆ to C₂₀ alkyl group, x is 10 to 20 and y is 80 to 120 may be used to make compositions in which, using 0.5 to 1.5% by weight additive based on the weight of coal, there is present from 67.5 to 70.5% weight of coal.

## Claims (Claims for the following Contracting State(s) : s BE, DE, FR, GB,. NL, SE)

1. A combustible composition of coal, water and surfactant comprising:
(i) from 30 to 90 parts by weight of pulverised coal,
(ii) from 0.05% to 3%, based on the dry weight of the pulverised coal, of a dispersing agent having the general formula wherein R is an alkyl group containing from 5 to 22 carbon atoms, or an alkylphenyl group in which the alkyl group contains from 5 to 22 carbon atoms,
x is an integer from 3 to 30, and
y is an integer and is at least 10, with the proviso that when R is a nonylphenyl group and x has a value of 8, the value of y is other than 20; and when R is a dinonylphenyl group and x has a value of 16, the value of y is other than 20; and
(iii) sufficient water to bring the total composition weight to 100 parts.

2. A composition according to claim 1 in which y is from 10 to 150.

3. A composition according to claim 1 or claim 2 in which the particle size of the coal is such that at least 80% of the particles are below 75 micrometres.

4. A composition according to any one of claims 1 to 3 in which x is from 10 to 20.

5. A composition according to any one of claims 1 to 4 in which y is from 80 120.

6. A composition according to any one of claims 1 to 5 in which R is an alkyl group.

7. A composition according to claim 6 in which R is an alkyl group containing from 16 to 20 carbon atoms.

8. A composition according to claim 7 which comprises:
(i) from 67.5 to 70.5% by weight of pulverised coal,
(ii) from 0.5 to 1.5%, based on the dry weight of the coal of a dispersing agent of formula (1) wherein
R is an alkyl group containing from 16 to 20 carbon atoms
x is from 10 to 20
y is from 80 to 120
(iii) sufficient water to bring the total composition weight to 100 parts.

9. A method of preparing a composition according to any one of claims 1 to 8 by the steps of:
(a) dissolving or dispersing the dispersing agent in water,
(b) adding the pulverised coal, and
(c) mixing the composition to produce the dispersion.

## Claims (Claims for the following Contracting State(s) : IT)

1. A combustible composition of coal, water and surfactant comprising:
(i) from 30 to 90 parts by weight of pulverised coal,
(ii) from 0.05% to 3%, based on the dry weight of the pulverised coal of a dispersing agent having the general formula wherein R is an alkyl group containing from 5 to 22 carbon atoms, or an alkylphenyl group in which the alkyl group contains from 5 to 22 carbon atoms,
x is an integer from 3 to 30, and
y is an integer and is at least 10, and
(iii) sufficient water to bring the total composition weight to 100 parts.

2. A composition according to claim 1 in which y is from 10 to 150.

3. A composition according to claim 1 or claim 2 in which the particle size of the coal is such that at least 80% of the particles are below 75 micrometres.

4. A composition according to claim 3 which comprises:
(i) from 67.5 to 70.5% by weight of pulverised coal,
(ii) from 0.5 to 1.5%, based on the dry weight of the coal of a dispersing agent of formula (I) wherein
R is an alkyl group containing from 16 to 20 carbon atoms
x is from 10 to 20
y is from 80 to 120
(iii) sufficient water to bring the total composition weight to 100 parts.

5. A method of preparing a composition according to any one of claims 1 to 4 by the steps of:
(a) dissolving or dispersing the dispersing agent in water,
(b) adding the pulverised coal, and
(c) mixing the composition to produce the dispersion.

## Patentansprüche (Patentansprüche für folgende(n) Vertragsstaat(en) : BE, DE, FR, GB, NL, SE)

1. Brennbare Zusammensetzung aus Kohle, Wasser und oberflächenaktivem Mittel, die folgendes umfaßt:
a) 30 bis 90 Gewichtsanteile an pulverisierter Kohle,
b) 0,05 bis 3%, bezogen auf das Trockengewicht der pulverisierten Kohle, eines Dispersionsmittels mit der allgemeinen Formel in der
R eine Alkylgruppe mit 5 bis 22 Kohlenstoffatomen, oder eine Alkylphenylgruppe ist, in der die Alkylgruppe 5 bis 22 Kohlenstoffatome enthält,
x eine ganze Zahl von 3 bis 30 ist, und
y eine ganze Zahl und mindestens 10 ist, mit der Maßgabe, daß wenn R eine Nonylphenylgruppe ist und x den Wert 8 besitzt, sich der Wert von y von 20 unterscheidet; und daß, wenn R eine Dinonylphenylgruppe ist und x den Wert 16 besitzt, sich der Wert von y von 20 unterscheidet; und
c) genügend Wasser, um das Gesamtgewicht der Zusammensetzung auf 100 Teile zu bringen.

2. Zusammensetzung nach Anspruch 1, in der y 10 bis 150 ist.

3. Zusammensetzung nach Anspruch 1 oder 2, in der die Teilchengröße der Kohle so bemessen ist, daß mindestens 80% der Teilchen kleiner als 75 Mikrometer sind.

4. Zusammensetzung nach einem der Ansprüche 1 bis 3, in der x 10 bis 20 ist.

5. Zusammensetzung nach einem der Ansprüche 1 bis 4, in der y 80 bis 120 ist.

6. Zusammensetzung nach einem der Ansprüche 1 bis 5, in der R eine Alkylgruppe ist.

7. Zusammensetzung nach Anspruch 6, in der R eine Alkylgruppe mit 16 bis 20 Kohlenstoffatomen ist.

8. Zusammensetzung nach Anspruch 7, die folgendes umfaßt:
a) 67,5 bis 70,5 Gew.-% an pulverisierter Kohle,
b) 0,5 bis 1,5%, bezogen auf das Trockengewicht der Kohle eines Dispersionsmittels mit der Formel (1), in der
R eine Alkylgruppe mit 16 bis 20 Kohlenstoffatomen ist,
x 10 bis 20 ist
y 80 bis 120 ist,
c) genügend Wasser, um das Gesamtgewicht der Zusammensetzung auf 100 Teile zu bringen.

9. Verfahren zur Herstellung einer Zusammensetzung nach einem der Ansprüche 1 bis 8, das folgende Schritte umfaßt:
a) Lösung oder Dispergieren des Dispersionsmittels in Wasser,
b) Zugeben der pulverisierten Kohle, und
c) Vermischen der Zusammensetzung zur Herstellung der Dispersion.

## Patentansprüche (Patentansprüche für folgende(n) Vertragsstaat(en) : IT)

1. Brennbare Zusammensetzung aus Kohle, Wasser und oberflächenaktivem Mittel, die folgendes umfaßt:
a) 30 bis 90 Gewichtsteile an pulverisierter Kohle,
b) 0,05 bis 3%, bezogen auf das Trockengewicht der pulverisierten Kohle eines Dispersionsmittels mit der allqemeinen Formel: in der
R eine Alkylgruppe mit 5 bis 22 Kohlenstoffatomen, oder eine Alkylphenylgruppe ist, in der die Alkylgruppe 5 bis 22 Kohlenstoffatome enthält,
x eine ganze Zahl von 3 bis 30 ist, und
y eine ganze Zahl und mindestens 10 ist, und
c) genügend Wasser, um das Gesamtgewicht der Zusammensetzung auf 100 Teile zu bringen.

2. Zusammensetzung nach Anspruch 1, in der y 10 bis 150 ist.

3. Zusammensetzung nach Anspruch 1 oder 2, in der die Teilchengröße der Kohle so beschaffen ist, daß mindestens 80% der Teilchen kleiner als 75 Mikrometer sind.

4. Zusammensetzung nach Anspruch 3, die folgendes umfaßt:
a) 67,5 bis 70,5 Gew.-% an pulverisierter Kohle,
b) 0,5 bis 1,5%, bezogen auf das Trockengewicht der Kohle eines Dispersionsmittels der Formel (I), in der
R eine Alkylgruppe mit 16 bis 20 Kohlenstoffatomen ist,
x 10 bis 20 ist,
y 80 bis 120 ist,
c) genügend Wasser, um das Gesamtgewicht der Zusammensetzung auf 100 Teile zu bringen.

5. Verfahren zur Herstellung einer Zusammensetzung nach einem der Ansprüche 1 bis 4, das folgende Schritte umfaßt:
a) Lösen oder Dispergieren des Dispersionsmittels in Wasser,
b) Zugeben der pulverisierten Kohle, und
c) Vermischen der Zusammensetzung zur Herstellung der Dispersion.

## Revendications (Revendications pour l'(les) Etat(s) contractant(s) suivant(s) : BE, DE, FR, GB, NL, SE)

1. Composition de combustible à base de charbon, d'eau et d'un surfactant, comprenant: '
(i) 30 à 90 parties en poids de charbon pulvérisé,
(ii) 0,05% à 3%, sur la base du poids sec du charbon pulvérisé, d'un agent de dispersion répondant à la formule générale dans laquelle R est un groupe alkyle contenant 5 à 22 atomes de carbone, ou un groupe alkylphényle dans lequel le groupe alkyle contient 5 à 22 atomes de carbone,
x est un nombre entier de 3 à 30, et
y est un nombre entier et est au moins égal à 10, sous réserve que, lorsque R est un groupe nonylphényle et x est égal à 8, la valeur de y est différente de 20; et, lorsque R est un groupe dinonylphényle et x est égal à 16, la valeur de y est différente de 20; et
(iii) une quantité d'eau suffisante pour porter le poids de la composition totale à 100 parties.

2. Composition suivant la revendication 1, dans laquelle y a une valeur de 10 à 150.

3. Composition suivant la revendication 1 ou la revendication 2, dans laquelle le diamètre des particules du charbon est choisi de manière qu'au moins 80% des particules aient un diamètre inférieur à 75 micromètres.

4. Composition suivant l'une quelconque des revendications 1 à 3, dans laquelle x a une valeur de 10 à 20.

5. Composition suivant l'une quelconque des revendications 1 à 4, dans laquelle y a une valeur de 80 à 120.

6. Composition suivant l'une quelconque des revendications 1 à 5, dans laquelle R est un groupe alkyle.

7. Composition suivant la revendication 6, dans laquelle R est un groupe alkyle contenant 16 à 20 atomes de carbone.

8. Composition suivant la revendication 7, qui comprend:
(i) 67,5 à 70,5% en poids de charbon pulvérisé,
(ii) 0,5 à 1,5%, sur la base du poids sec du charbon, d'un agent de dispersion répondant à la formule (I) dans laquelle R est un groupe alkyle contenant 16 à 20 atomes de carbone, x a une valeur de 10 à 20, ya une valeur de 80 à 120,
(iii) une quantité d'eau suffisante pour porter le poids de la composition totale à 100 parties.

9. Procédé de préparation d'une composition suivant l'une quelconque des revendications 1 à 8, comprenant les étapes consistant:
(a) à dissoudre ou disperser l'agent de dispersion dans l'eau,
(b) à ajouter le charbon pulvérisé, et
(c) à mélanger la composition pour produire la dispersion.

## Revendications (Revendications pour l'(les) Etat(s) contractant(s) suivant(s) : IT)

1. Composition de combustible à base de charbon, d'eau et d'un surfactant, comprenant:
(i) 30 à 90 parties en poids de charbon pulvérisé,
(ii) 0,05% à 3%, sur la base du poids sec du charbon pulvérisé, d'un agent de dispersion, répondant à la formule qénérale dans laquelle R est un groupe alkyle contenant 5 à 22 atomes de carbone, ou un groupe alkylphényle dans lequel le groupe alkyle contient 5 à 22 atomes de carbone,
x est un nombre entier de 3 à 30, et
y est un nombre entier et est au moins égal à 10, et
(iii) une quantité d'eau suffisante pour porter le poids de la composition totale à 100 parties.

2. Composition suivant la revendication 1, dans laquelle y a une valeur de 10 à 150.

3. Composition suivant la revendication 1 ou la revendication 2, dans laquelle le diamètre des particules de charbon est choisi de manière qu'au moins 80% des particules aient un diamètre inférieur à 75 micromètres.

4. Composition suivant la revendication 3, qui comprend:
(i) 67,5 à 70,5% en poids de charbon pulvérisé,
(ii) 0,5 à 1,5%, sur la base du poids sec du charbon, d'un agent de dispersion répondant à la formule (I) dans laquelle
R est un groupe alkyle contenant 16 à 20 atomes de carbone,
x a une valeur de 10 à 20,
y a une valeur de 80 à 120,
(iii) une quantité d'eau suffisante pour porter le poids de la composition totale à 100 parties.

5. Procédé de préparation d'une composition suivant l'une quelconque des revendications 1 à 4, comprenant les étapes consistant:
(a) à dissoudre ou à disperser l'agent de dispersion dans l'eau,
(b) à ajouter le charbon pulvérisé, et
(c) à mélanger la composition pour produire la dispersions.
